

March 2, 1948.

T. O. THEOBALD

2,437,177

METHOD OF CASTING AND APPARATUS THEREFOR

Filed Oct. 28, 1944



Fig. 4.

Fig. 3



Fig. 1.



Fig. 5.

Fig. 2.

INVENTOR.

T. O. Theobald.

BY Edwin C. McRae

R. J. Harris

ATTORNEYS.

## UNITED STATES PATENT OFFICE

2,437,177

METHOD OF CASTING AND APPARATUS  
THEREFOR

Thomas O. Theobald, Royal Oak, Mich.

Application October 28, 1944, Serial No. 560,784

3 Claims. (Cl. 22—184)

1

This invention relates to a new method of metal casting, the specific improvement being the provision of means whereby the risers and runners associated with such casting may be more conveniently removed therefrom. It is usual foundry practice to provide at least one gate in each mold into which gate the molten metal is poured, and which gate is connected to the article cavity by means of runners. Risers extend upwardly from the mold cavity into which a relatively large amount of metal can rise to feed the casting proper as the metal in the casting shrinks as it solidifies. The number and size of risers required for any particular casting varies with the shape of the casting and with the type of metal used. For example, comparatively few risers are required when the casting is to be made of iron; whereas, when casting of aluminum, or magnesium, many risers of large cross section are required to compensate for shrinkage in the casting. Furthermore, few risers are required where the casting is of uniform wall thickness; whereas, a riser must be placed opposite a thick boss or the like, as such boss cools slower than the walls and must be fed by a liquid source as it cools.

A riser to function satisfactorily must be designed with sufficient cross sectional area, so that the metal in the casting will have completely solidified before solidification of the metal in the riser. If the riser solidifies before any portion of the casting, then shrinkage defects inevitably occur in the casting. From the foregoing, it will be apparent that when forming casting having comparatively thick bosses or sections, the risers must have a fairly large cross sectional area—otherwise the riser will solidify before the thick section of the casting.

One disadvantage of providing risers of large cross section is that the riser must be sawed or cut from the casting in cleaning up the casting prior to the machine operations proper. This requires considerable labor. Furthermore, where the riser is positioned beneath a flange or the like, great difficulty is usually experienced in removing the riser, as a saw cannot be inserted at the base of the riser.

The object of this invention is to provide a method of casting whereby the riser may be designed with a relatively large cross sectional area, but still may be readily removed from the casting by striking it a sharp blow.

A further object of my invention is to provide a relatively simple snagging washer which is cast in the riser whereby the above objects are readily accomplished.

With these and other objects in view, my invention consists in the various steps of my improved process and in my improved article as described in this specification, claimed in my

claims and shown in the accompanying drawings, in which:

Figure 1 is a plan view of a portion of internal-combustion engine cylinder head casting having risers connected extending upwardly from the casting proper.

Figure 2 is a sectional view, taken on the line 2—2 of Figure 1.

Figure 3 is a full size view of one of the risers shown in Figure 2—this view also being taken on line 2—2 of Figure 1.

Figure 4 is a plan view of a snagging plate or washer which is adapted to be cast in the base of the riser, and

Figure 5 is a fragmentary sectional view, similar to Figure 3, but shows a modified form of my snagging washer.

Referring to the accompanying drawings, I have used the numeral 10 to indicate a cylinder head casting proper, from which a riser 11 extends, the riser being connected thereto by a means of a pair of necks 12. In the construction shown, the riser 11 is connected to the casting proper by two necks 12, but this is done only for convenience as in most cases a single neck is ample. However, in forming the casting shown, it is necessary to place a riser directly above each of the closely spaced valve guide bosses 13. These bosses have large cross sectional areas, and a riser is required for each boss to supply metal as they cool. In this case the individual risers are so close together that for convenience each two adjacent risers are combined to form a single riser casting. However, due to the provision of the two necks 12, the single riser feeds both of the adjacent bosses the same as it would two separate risers.

It may be noted from Figure 3 that each of the necks 12 is provided with an annular shoulder 14, spaced just above the casting proper. The diameter of the riser neck must be made sufficiently large so that the metal in the boss 13 will have solidified before the metal in the neck portion solidifies, otherwise the molten metal in the riser will not feed down into the casting. When the neck 12 is designed with a sufficiently large diameter to accomplish the above-mentioned purpose, it usually happens that the neck has such structural strength that it cannot be broken from the casting without destroying the adjacent part of the casting. If an attempt is made to break the riser off by striking it a blow, it often happens that the casting is broken instead, thereby destroying the entire casting.

In this invention, I provided means for reducing the cross sectional area of each neck 12 as far as its structural strength is concerned, while maintaining its initially large cross sectional area for the transfer of heat therethrough. It should be kept in mind that a riser neck of

the same cross sectional area—as a boss on the casting—will remain liquid until after the boss solidifies, because of the flow of heat into the neck from the comparatively large body of metal in the riser proper. The riser neck loses heat to the adjacent mold as fast as does the casting, but the liquid metal in the riser supplies heat to the neck to cause it to cool slower than the adjacent portion of the casting.

The unique feature of this invention is that the means provided for reducing the cross sectional area of the riser does not retard the transfer of heat to the neck and does not absorb any appreciable heat itself, so that no chilling effect is produced thereby. I accomplished this by providing a washer 15 formed of very thin metal as illustrated in Figure 4. The outside diameter of the washer is just large enough to be easily inserted into the neck 12 and to rest upon the shoulder 14. The opening 19 in the washer is considerably smaller than the diameter of the neck 12. Each washer 15 is provided with four tongues 16, which are stamped from the material of the washer and which project from the periphery about one 32nd of an inch. The tongues normally lie in the same plane as the washer, but when it is inserted into position upon the shoulder 14, the tongues projecting beyond the periphery of the washer are sprung upwardly to some extent, as shown in Figure 3. The washer is thus prevented from becoming loose in the mold and possibly being dislocated, as the metal is poured. The tongues extend about two thirds of the way through the washer so that they may be sprung upwardly by the comparatively soft core sand walls of the mold.

It is essential in carrying out this invention that the washer 15 be formed of material having a relatively high heat transfer coefficient and that it be constructed of relatively thin material, so that the restriction to the transfer of heat from the riser will be a minimum. I have found that in pouring aluminum or magnesium castings, it is preferable to make the washers 15 from a relatively thin sheet steel stock of a thickness of about .010". This stock is known as shim stock. The opening in the washer 15 in the casting shown is about one-quarter of an inch smaller than the diameter of the neck 12. It has been calculated that a minimum riser neck area of 1 $\frac{1}{8}$ " diameter is necessary to maintain fluidity in the riser during the solidification of the casting bosses shown. The opening in the washer 15, however, is only 1 $\frac{1}{8}$ " in diameter. This reduction in the effective structural cross section of the riser directly reduces the strength of the riser by 30%. However, the greatest gain results from the localizing of the stresses along the bottom of the narrow groove formed by the thin washer. This acts as a crack in the riser and causes the riser to break off by an impact force of only a fraction of that required to break off a riser of 1 $\frac{1}{8}$ " uniform diameter. In production, the force required to break off the riser in the casting shown, is only about one third that required to break off a riser formed without the washer 15.

In carrying out my improved method of casting, a mold is formed having cavities therein corresponding to the pouring gate, runners, casting proper and the risers. This mold is constructed in the conventional manner and forms a part of my invention only in combination with my snagging washer 15. The mold proper has not, therefore, been illustrated in the drawings.

After the mold is formed and the washers 15

are in place, metal is poured therein, which metal flows up through the casting cavity proper and then through the necks 12 to fill the risers 11. As the casting gradually solidifies, metal from the riser 17 is drawn down through the necks 12 to compensate for shrinkage in the bosses 13. Due to the fact that the heat radiation from the neck portion 12 is proportional to the area of the neck and that heat is added to the neck from the metal in the riser, the metal therein will stay fluid until the casting is completely solidified. Subsequently, the neck 12 and the riser will solidify, at which time casting can be removed from the sand. The risers are then removed from the casting proper by simply striking the riser a sharp blow with a hammer. The washers 15 do not form a bond with the metal of the casting, so that it is only necessary to break the portion of the riser within the opening 17. Furthermore, inasmuch as the washer forms a sharp crevice in the riser, the impact force supplied to the riser receiving the blow is localized at this point, so that the riser breaks off with only a fraction of the force otherwise required.

It will be noted that the casting shown has a flange forming a part thereof so spaced that the juncture of the riser with the casting is obstructed by this flange. The riser in this case could not, therefore, be conveniently removed by sawing through the necks 12 with the usual snagging band saw. This example illustrates an important feature of my invention, as the riser may be broken as disclosed herein very close to the casting without interference from associated parts of the casting.

I have heretofore referred only to the casting of aluminum, magnesium, and the like. However, iron may be cast with my improved method, but the washer must be formed so that it will not melt when in contact with the hot metal. This can be accomplished, as shown in Figure 5, by coating the washer herein numbered 17 with a ceramic material 18, which fuses at a temperature above that of the metal being poured. In some cases, the washer may be formed from a higher melting alloy with good results.

It should be kept in mind that while I have shown my invention as applied to a riser, the invention may be equally advantageous for use in removing gates, sprues, runners, etc., from the associated casting. In the attached claims the term riser is therefore meant to include any part of the rough casting which is added thereto for the purpose of pouring the casting proper.

Some changes may be made in the shape of the washer 15, without departing from this invention, as it may in some cases only be necessary to insert a thin strip of shim stock along one edge of a square riser. Furthermore, some changes may be made in the mold structure and in the several steps comprising my improved method, without departing from the spirit of my invention, and it is my intention to cover by my claims such changes as may reasonably be included within the scope thereof.

I claim as my invention:

1. A snagging washer to be inserted in a riser of a casting mold comprising, a flat thin sheet metal stamping formed of shim stock having an opening therein, said opening proportioned to reduce the cross sectional area of the riser to about two-thirds, and a plurality of tongues stamped from the material of said washer, said tongues projecting slightly beyond the periphery of the

washer and extending back into the body of the washer a major portion of the distance therethrough, for the purpose described.

2. A snagging member to be inserted in a riser of a casting mold, comprising, a flat thin sheet metal stamping formed of shim stock proportioned to reduce the cross sectional area of a riser to about two-thirds, and a plurality of tongues stamped from the material of said member, said tongues projecting slightly beyond the 10 periphery of the member and extending back into the body of the member a major portion of the distance therethrough, for the purpose described.

3. A method of casting articles of nonferrous metals comprising forming a mold having cavities therein corresponding to the casting proper and to a riser, respectively, and inserting in the passageway connecting the casting proper and the riser a snagging washer made of a flat, thin, sheet metal stamping having an opening therein, 20

5 said opening being proportioned to reduce the cross sectional area of the riser to about two thirds, and having a plurality of tongues stamped from the material of said washer, said tongues projecting slightly beyond the periphery of the washer and extending back into the body of the washer a major portion of the distance therethrough.

THOMAS O. THEOBALD.

#### REFERENCES CITED

The following references are of record in the file of this patent:

#### UNITED STATES PATENTS

| Number    | Name     | Date          |
|-----------|----------|---------------|
| 388,336   | Boulton  | Aug. 21, 1888 |
| 855,396   | Foreman  | May 28, 1907  |
| 900,970   | Washburn | Oct. 13, 1908 |
| 2,334,929 | Hone     | Nov. 23, 1943 |